

# UNITED STATES PATENT OFFICE.

JOHN A. M. LEWIS AND FRED A. WAGER, OF SALT LAKE CITY, UTAH.

## FURNITURE-POLISH.

1,121,590.

Specification of Letters Patent. Patented Dec. 15, 1914.

No Drawing.

Application filed November 25, 1913. Serial No. 803,062.

*To all whom it may concern:*

Be it known that we, JOHN A. M. LEWIS and FRED A. WAGER, citizens of the United States, residing at Salt Lake City, in the county of Salt Lake and State of Utah, have invented certain new and useful Improvements in Furniture-Polishes, of which the following is a specification.

Our invention relates to furniture polishes, and has for its object to provide a furniture polish which will dissolve and cut the grease and dirt from used furniture and restore the finish and luster thereto.

A further object is to provide a furniture polish which dries quickly and leaves no gummy, sticky or dust collecting particles on the furniture treated.

A further object is to preserve the finish of new furniture.

These objects we accomplish with the new and useful composition of matter hereinafter described, in the proportions in which they are used and in the novel manner in which they are compounded.

In our polish we use two parts of mineral oil, preferably paraffin oil, to one part of hydrochloric acid. When mixed and thoroughly agitated the acid will cut the grease and gummy particles in the oil. This agitated mixture is then allowed to stand until the oil separates out, and said grease and gummy parts of the oil with the acid settle at the bottom. This precipitation takes from one to three hours. The oil at the top

is then drawn or poured off and the precipitates, the grease and gummy parts with the acid are thrown away. We then mix one part of the retained and treated oil with two parts of commercial turpentine. Our process may be varied to the extent of adding the turpentine to the previous mixture before the agitation and precipitation has occurred, as the precipitation and result will be the same. To every

gallon of this mixture, of oil and turpentine, we add one pound of commercial chlorid of lime and again thoroughly agitate. After this agitation the mixture is allowed to stand until the calcium hydroxid settles and

is precipitated and leaves the liquid clear of sediment. The liquid portion is then drawn or poured off and filtered through felt, filter paper or any of the well known filters, to insure that there is none of the lime particles or other gritty substances remaining in the polish. We thus prepare and provide a polishing liquid having a light amber color and with a specific gravity of 1.1165, that will cut the grease and dirt from furniture and when rubbed briskly with cloth will dry quickly and leave the furniture treated therewith ready for immediate use with the polish restored to its original finish.

Having thus described our invention we desire to secure by Letters Patent and claim:

1. The herein described polishing compound consisting of clarified paraffin oil one part; and turpentine two parts.

2. A polishing compound consisting of clarified mineral oil having a paraffin base one part; and turpentine two parts.

3. A polishing liquid of light amber color and having a specific gravity of 1.1165 consisting of mineral oil having a paraffin base one part and turpentine two parts.

4. The process of compounding furniture polish which consists of agitating and precipitating two parts of paraffin oil with one part of hydrochloric acid, and retaining only the oil, to which two parts of turpentine is added; and deodorizing and clarifying with chlorid of lime, as herein described.

5. The process of compounding furniture polish which consists of agitating and precipitating two parts of paraffin oil, with one part of hydrochlorid acid, and retaining only the oil, to which two parts of turpentine is added, this mixture is then deodorized and clarified.

In testimony whereof we have affixed our signatures in presence of two witnesses.

JOHN A. M. LEWIS.  
FRED A. WAGER.

Witnesses:

SAM RANEY,  
W. R. WILLIAM.